

[54] N-ALKYL MORPHOLINE TREATMENT OF  
A SELENIUM-CONTAINING  
PHOTOCONDUCTIVE LAYER[75] Inventors: **Bela Telek; Thomas Skaper**, both of  
Penfield, N.Y.[73] Assignee: **Xerox Corporation**, Stamford,  
Conn.[22] Filed: **Oct. 19, 1973**[21] Appl. No.: **408,248**[52] U.S. Cl. .... **96/1.5, 117/201, 117/215**[51] Int. Cl. .... **G03g 5/00, G03g 5/02**[58] Field of Search ..... **96/1.5, 1.8; 117/215, 201**

## [56] References Cited

## UNITED STATES PATENTS

|           |         |                   |          |
|-----------|---------|-------------------|----------|
| 3,355,289 | 11/1967 | Hall et al. ....  | 96/1.5 X |
| 3,501,294 | 3/1970  | Joseph ....       | 96/1.5 X |
| 3,713,820 | 1/1973  | Champ et al. .... | 96/1.5   |
| 3,748,128 | 7/1973  | McNally ....      | 96/1.5 X |

## FOREIGN PATENTS OR APPLICATIONS

|           |        |            |        |
|-----------|--------|------------|--------|
| 43-16,198 | 7/1968 | Japan .... | 96/1.5 |
|-----------|--------|------------|--------|

*Primary Examiner*—David Klein*Assistant Examiner*—John R. Miller*Attorney, Agent, or Firm*—James J. Ralabate; James P. O'Sullivan; John H. Faro

[57]

## ABSTRACT

Methods for conditioning electrophotographic imaging members wherein the photoconductive imaging layer comprises amorphous selenium or selenium alloys. According to this method, the photoconductive imaging layer is treated with a liquid containing at least one N-substituted morpholine compound of the formula



wherein R is a saturated aliphatic hydrocarbon radical having in the range of from about 8 to about 30 carbon atoms.

The application of such materials to the imaging layer of the imaging member provides said layer with a finish which is capable of protecting said layer from abrasion and the adverse effects of humidity while at the same time enhancing charge acceptance thus improving solid density development.

34 Claims, No Drawings

**N-ALKYL MORPHOLINE TREATMENT OF A  
SELENIUM-CONTAINING PHOTOCONDUCTIVE  
LAYER**

**BACKGROUND OF THE INVENTION**

**1. Field of the Invention**

This invention relates to a method, an imaging member prepared according to said method and the use of said imaging member in an imaging process. More specifically, this invention involves methods for preconditioning and reconditioning the imaging layer of an electrophotographic imaging member, the overcoated electrophotographic imaging member resulting from such treatment and an imaging process employing said overcoated electrophotographic imaging member.

**2. Description of the Prior Art**

The formation and development of images on an imaging layer of photoconductive materials by electrostatic means is well known. The best known of the commercial processes, more commonly known as xerography, involves forming a latent electrostatic image on the imaging layer of imaging member by first uniformly electrostatically charging the surface of the imaging layer in the dark and then exposing this electrostatically charged surface to a light and shadow image. The light struck areas of the imaging layer are thus rendered conductive and the electrostatic charge selectively dissipated in these irradiated areas. After the photoconductor is exposed, the latent electrostatic image on this image bearing surface is rendered visible by development with finely divided colored electroscopic powder material, known in the art as "toner". This toner will be principally attracted to those areas on the image bearing surface which retain the electrostatic charge and thus form a visible powder image.

The developed image can then be read or permanently affixed to the photoconductor in the event that the imaging layer is not to be reused. This latter practice is usually followed with respect to the binder-type photoconductive films where the photoconductive layer is also an integral part of the finished copy.

In so-called "plain paper" copying systems, the latent image can be developed on the imaging surface of a reusable photoconductor or transferred to another surface, such as a sheet of paper, and thereafter developed. When the latent image is developed on the imaging surface of a reusable photoconductor, it is subsequently transferred to another substrate and then permanently affixed thereto. Any one of a variety of well known techniques can be used to permanently affix the toner image to the transfer sheet, including overcoating with transparent films and solvent or thermal fusion of the toner particles to the supportive substrate.

Prior to recycling of the photoreceptor, untransferred toner particles adhering to the surface of the imaging layer of the photoreceptor must be removed in order to prevent deterioration in quality in subsequent copies. Various devices have been employed in the past for removal of these toner residues from the surface of the photoreceptor. Typical of such cleaning means include rotating brushes of the type disclosed in U.S. Pat. No. 2,832,977; cleaning webs of the type disclosed in U.S. Pat. No. 3,186,833; and blade cleaning devices of the type disclosed in U.S. Pat. No. 3,634,077. The relative efficiency which these cleaning means remove toner residues is often dependent upon a number of variables; including the presence of an additive in the

developer composition, the presence of an overcoating on the photoreceptor surface, the relative electrostatic attraction of the toner to the photoreceptor surface and the physical force exerted by the cleaning means against the photoreceptor surface. Since the imaging surface of selenium photoreceptors are sensitive to abrasion the pressure contact between the above cleaning means and this surface must be kept to a minimum in order to prevent damage to the imaging surface. This frictional contact of the cleaning means against the photoreceptor surface can also result in erosion of the cleaning member, U.S. Pat. No. 3,682,689. The blade cleaning type device previously referred to is especially vulnerable to this type of wear. If the photoreceptor surface is somewhat irregular, especially if it has minute projections, the pressure contact of the leading edge of a blade cleaning means against this surface can result in the rapid deterioration of the cleaning blade. In order to minimize the possibility of this occurring, extreme care is exercised in the manufacture of photoreceptors. Such care must be exercised at all stages of preparation of this multilayer component since any defects in any of the underlying layers can be translated into a surface imperfection in the outer layer of photoconductive materials.

During servicing of heavily toner laden photoreceptors, it has been common practice to buff the photoreceptor surface with a pumicing agent in order to remove accumulated toner residues and thus restore the photoreceptor surface to its virgin state. Such pumicing agents are also used in the reconditioning of such photoreceptor surfaces in order to remove minor scratches which have developed over extended periods of use. These same buffering compounds are now being employed in the dressing of new photoreceptors in order to insure that any imperfections (especially minor projections) are removed prior to the installation of the photoreceptor into a copier employing a blade cleaning device. Unfortunately, a number of the commercial buffering compounds used in preconditioning and reconditioning selenium photoreceptors also contain residues which adhere to the imaging surface of the photoreceptor thereby impairing its electrophotographic properties. One type of residue which has proven to be particularly troublesome is glycerol monostearate. The extent to which this substance can disrupt the electrophotographic properties of the photoreceptor varies with the particular composition of the imaging layer of said photoreceptor. For example, where the photoconductive insulating layer comprises an arsenic-selenium alloy the effects of this substance on the photoreceptor are more pronounced.

It is, therefore, the principal object of this invention to provide a method for minimizing the adverse effect of the above and similar residues on photoconductive insulating layers comprising amorphous selenium or selenium alloys.

More specifically, it is the object of this invention to provide a method for preconditioning new electrophotographic imaging members wherein the photoresponsive layer comprises amorphous selenium or selenium alloys.

It is yet another object of this invention to provide a method for reconditioning used electrophotographic imaging members wherein the photoresponsive layer comprises amorphous selenium alloys.

It is yet a further object of this invention to provide the imaging surface of said imaging member with an overcoating during preconditioning which improves both abrasion and moisture resistance in addition to enhancing solid density development.

It is yet a further object of this invention to provide the imaging surface of said imaging member with an overcoating during reconditioning which improves both abrasion and moisture resistance in addition to enhancing solid density development.

Still yet a further object of this invention is to provide an overcoated imaging member wherein said overcoating improves abrasion and moisture resistance in addition to enhancing solid density development.

Still yet a further object of this invention is to provide an electrophotographic imaging method employing the above overcoated imaging member.

#### SUMMARY OF THE INVENTION

The above and related objects are achieved by providing a method for conditioning the amorphous selenium or selenium alloy photoconductive layer of an electrophotographic imaging member. According to this method, an imaging member having a photoconductive imaging layer comprising amorphous selenium or selenium alloy is treated with a conditioning effect amount of at least one N-substituted morpholine compound of the formula



wherein, R is a saturated aliphatic hydrocarbon radical having in the range of from about 8 to 30 carbon atoms.

In the preferred embodiments of this invention, a dilute solution of one or more of the above compounds is applied to the amorphous selenium or selenium alloy imaging layer of the photoreceptor and then excess solution removing after a predetermined period of time. The preferred compound used in the methods of this invention is N-lauryl-morpholine.

#### DESCRIPTION OF THE INVENTION INCLUDING PREFERRED EMBODIMENTS

The electrophotographic imaging member which can be treated in accord with the methods of this invention comprises a conductive substrate having coated on at least one surface thereof a photoconductive film comprising amorphous selenium, a selenium alloy, or mixtures thereof. Any of the conductive substrates traditionally used in the preparation of electrophotographic imaging members are suitable for use in preparation of the overcoated electrophotographic imaging members of this invention. Such substrates can be flexible or inflexible; organic or inorganic; and transparent or opaque. Representative of substrates which have proven suitable for use in such devices include aluminum, nickel, chromium, polyethylene terephthalate overcoated with a thin metal film, or metalized plastic films. Ordinarily, prior to the deposition of the photoconductive insulating layer on such substrate, an interfacial barrier layer is deposited on such substrate in order to provide a blocking contact against premature injection of carriers from the conductive substrate into

the photoconductive insulating layer. This interfacial barrier layer can be an insulating material such as a dielectric film of an inorganic oxide. It is generally preferred that such interfacial barrier layers be capable of rectification. Once the conductive substrate has been prepared and an interfacial barrier layer formed thereon (where desired), the substrate is placed in a vacuum evaporation chamber and a photoconductive insulating layer of selenium, selenium alloy or mixtures thereof deposited on the appropriate surface of the substrate. Deposition of such photoconductive materials is allowed to proceed until the deposit forms a substantially uniform film having a thickness in the range of from about 0.1 to about 100 microns.

During the evaporation of such photoconductive materials, minute dust particles in the vacuum evaporation chamber can also codeposit along with the selenium on the conductive substrate, thus, forming blemishes in the photoconductive coating. In order to minimize the effect of such asperities, the photoconductive surface is gently buffed with a pumicing agent until such imperfections are substantially removed. As indicated previously, organic residues contained within these agents can adhere to the imaging surface of the photoconductive insulating layer and where not removed, can impair the electrophotographic properties of said imaging layer.

In order to both insure against such residue interference and enhance the abrasion resistance, moisture resistance and/or charge acceptance, a solution containing one or more of the aforescribed compounds is applied to the imaging layer of the photoreceptor in sufficient quantities to affect one or more of the above improvements. A typical solution of such conditioning agent should contain sufficient conditioning compound to impart the desired beneficial results and yet facilitate processing of the photoreceptor. For example, in the event that about 1 gram conditioning compound is dissolved in about 100 milliliters of appropriate solvent, the residence time of the conditioning solution on the imaging layer required to impart the desired beneficial results is quite extensive, generally in excess of about 20 minutes. Where the concentration of conditioning compound in the appropriate solvent is from about 5 to about 10 grams per 100 milliliters solvent, the residence time of the solution on the imaging layer need only be about 5 minutes in order to impart the desired beneficial finish. Where the concentration of conditioning compound is substantially in excess of 10 grams per 100 milliliters solvent, the increased viscosity of the conditioning solution creates problems in uniformity of application and penetration of the conditioning compounds into the microporous surface of the imaging layer. Solvents which are suitable for use as vehicles for dispensing the conditioning compounds on the imaging layer must be compatible with the imaging layer (not interfere with or bring about changes in the electronic and/or physical properties) and must also be compatible with the environment in which such conditioning takes place. Representative of solvents which are suitable for preparation of the conditioning solution include methanol, ethanol, n-propanol, isopropanol, and n-butanol.

Subsequent to preparation of the conditioning solution, it can be applied to the imaging layer of the imaging member by any one of a number of standard coating techniques including aerosol application or a wipe-

on application. Whatever the mode of application of the conditioning solution to the imaging layer that is ultimately selected, it must provide for the uniform coverage of the surface of the imaging layer with sufficient conditioning compound to effectively remove the organic buffering compound residues (if any), enhance abrasion resistance, enhance moisture resistance and/or enhance charge acceptance. In order to enhance one or more of these properties, it is not necessarily required that such treatments enhance all such properties. For example, where the conditioning compound has a relatively small aliphatic hydrogen substituent (8 carbon atoms), the relative abrasion resistance of the imaging layer is not enhanced to the extent it would be where such substituent has in excess of about 20 carbon atoms. However, charge acceptance is substantially improved where the imaging layer is conditioned with compounds having such relatively short chain hydrocarbon substituents.

Subsequent to application of a conditioning solution over substantially the entire imaging layer of an electrophotographic imaging member, the solution is allowed to saturate the surface of said imaging layer for a period of anywhere from about 3 to 10 minutes (preferably about 5 minutes). Subsequent to saturation of the photoreceptor, nonabsorbed and nonadsorbed conditioning materials are removed from said surface by wiping said surface with a soft, damp fabric or sponge. The wiper used in removing excess conditioning agent is ordinarily wetted with the same solvent vehicle used in application of the conditioning compounds to the imaging layer. After removal of excess conditioning compounds, the imaging surface is dried with a soft absorbent fabric or other suitable means. It is generally preferred that the solvents used in dispensing and removal of the conditioning compounds from the surface of the photoreceptor be highly volatile and thus capable of evaporation from said surface without any residual trace thereof remaining on said surface.

Conditioning of the drum in the manner described above does not alter the appearance of the imaging layer since the conditioning compounds are present in such small quantities and thus are not readily detectable except by sophisticated analytical techniques. For example, where an electrophotographic imaging member having an imaging layer of a surface area equal to about 3,000 square centimeters is conditioned in the manner described above, the quantity of conditioning compound capable of extraction from said layer is equal to about 0.6 to about 1.5 milligrams; or approximately 0.2 to about 0.5 micrograms per square centimeter. The presence of the conditioning compound on the imaging layer can be detected by infrared spectroscopy after 4,000 copies. In a typical evaluation of the efficacy of the conditioning procedure, an electrophotographic imaging member conditioned according to the method of this invention is placed in an electrostaticographic copier, and copy tested to 10,000 copies (2 copies per cycle of photoreceptor). The cleaning apparatus of this copier comprises a polyurethane blade which translates laterally across the surface of the photoreceptor. The developer composition used in this copier contains a nonsmearing additive intended to enhance removal of residual toner from the surface of the photoreceptor. Comparison of efficiency of cleaning both prior to and subsequent to conditioning of the imaging layer of the photoreceptor reveals a reduction of

about 70 percent in the frictional forces between the blade and the imaging layer. Comparison of charge acceptance of the conditioned and unconditioned portion of the photoreceptor reveals about a 10 percent increase in charge acceptance in the conditioned areas.

This treatment of selenium and selenium alloys photoreceptors provides the surface of said photoreceptor with a finish which substantially extends their useful lives in addition to reducing servicing requirements of both the photoreceptor and the cleaning means used in removal of toner residues from the imaging layer of said photoreceptor.

The examples which follow further define, describe and illustrate the methods of this invention. Apparatus and techniques used in these examples are standard or as hereinbefore described. Parts and percentages appearing in such examples are by weight unless stipulated otherwise.

#### EXAMPLE I

An electrophotographic imaging member having an imaging layer comprising an alloy of arsenic and selenium (65 percent by weight selenium to 35 percent by weight arsenic) is sectioned off and alternate sections conditioned with a solution comprising 5 percent N-laurylmorpholine in isopropyl alcohol. The conditioning solution is applied with a cotton cloth and allowed to reside on the photoreceptor for an interval of approximately 5 minutes prior to removal of excess conditioning compound with isopropyl alcohol. Subsequent to the removal of excess conditioning compounds, the photoreceptor is wiped dry with a soft cotton cloth in those areas where the conditioner was applied. Following conditioning, the photoreceptor is sensitized by charging with a positive corotron which is maintained at 8,000 volts. Measurement of the surface potential on the photoreceptor indicates that those areas which have been conditioned with the N-laurylmorpholine can support a surface potential of about 800 volts whereas those regions on the photoreceptor not so conditioned can only support a surface potential of about 700 volts. The photoreceptor is then placed in a standard Xerox 4,000 copier and several copies prepared therefrom. Examination of these copies clearly indicates that those areas of the photoreceptor which have been conditioned with the N-laurylmorpholine do produce copies of improved density even after 4,000 copying cycles. The photoreceptor is then removed and examined. It appears that the conditioned sections of the photoreceptor are substantially freer of toner residues than those sections not treated with the conditioning solution; thus, indicating more efficient blade cleaning action.

#### EXAMPLE II

The procedures of Example I are repeated except for the substitution of a conditioning solution containing about 1 gram N-laurylmorpholine per 100 milliliters isopropyl alcohol. Although some improvement in charge acceptance and solid density development are noted, it is apparent that the extent of improvement falls considerably short of that obtained in Example I.

#### EXAMPLE III

The procedures of Example II are repeated except that the conditioning solution is allowed to remain on the imaging layer of the electrophotographic imaging

member for a period of about 25 minutes prior to removal of nonabsorbed compounds with isopropyl alcohol. The charge acceptance and solid density development are improved over that attained in Example II but still are not comparable to that of Example I.

#### EXAMPLE IV

The procedures of Example I are repeated except for the substitution of a conditioning solution containing 15 grams N-lauryl morpholine per 100 grams isopropyl alcohol. Due to the increased viscosity of this conditioning solution over that of Example I, the application of a uniform film on the imaging layer is somewhat more difficult. Following removal of excess conditioning compounds, the imaging layer is evaluated in the same manner as in Example I. Both charge acceptance and solid density development are inferior to that of Example I. It is believed that due to the increase in viscosity, the conditioning compound does not wet the imaging layer as efficiently as does the conditioning solution of Example I. Thus, the effectiveness of the conditioning compound is substantially reduced, resulting in less efficient and complete absorption and adsorption on the imaging layer.

#### EXAMPLE V

The procedure of Example I is repeated except for the substitution of N-capryl-morpholine for N-lauryl-morpholine.

#### EXAMPLE VI

The procedure of Example I is repeated except for the substitution of N-capryl-morpholine for N-lauryl-morpholine.

#### EXAMPLE VII

The procedure of Example I is repeated except for the substitution of N-myristyl-morpholine for N-lauryl-morpholine.

#### EXAMPLE VIII

The procedure of Example I is repeated except for the substitution of N-palmityl-morpholine for N-lauryl-morpholine.

#### EXAMPLE IX

The procedure of Example I is repeated except for the substitution of N-stearyl-morpholine for N-lauryl-morpholine.

#### EXAMPLE X

The procedure of Example I is repeated except for the substitution of N-arachidyl-morpholine for N-lauryl-morpholine.

#### EXAMPLE XI

The procedure of Example I is repeated except for the substitution of N-behenyl-morpholine for N-lauryl-morpholine.

#### EXAMPLE XII

The procedure of Example I is repeated except for the substitution of N-lignoceryl-morpholine for N-lauryl-morpholine.

#### EXAMPLE XIII

The procedure of Example I is repeated except for

the substitution of N-cerotyl-morpholine for N-lauryl-morpholine.

#### EXAMPLE XIV

In order to determine quantitatively the extent to which N-lauryl-morpholine reduces the frictional force between the cleaning blade and the photoreceptor surface in Example I, the photoreceptor is removed from the copier and installed in a testing fixture. A portion of the polyurethane blade is removed from the copier and installed in a holder in the testing fixture. The combined weight of the blade and holder is approximately 60 grams. The blade is rested on the surface of the photoreceptor (blade area in contact with photoreceptor = 20 millimeters  $\times$  2.2 millimeters). As the blade is drawn across the surface of the photoreceptor, the force required to advance the blade increases as the blade traverses from the conditioned to the unconditioned portions of the photoreceptor. Such change in force is measured on a simple spring scale (Ohaus, Dial Type scale) which is attached to the blade holder. From such measurements, the coefficient of friction ( $\mu$ ) for the conditioned areas of the drum is calculated to be in the range of from about 0.025 to 0.030; and the coefficient of friction for the unconditioned areas of the drum calculated to be in the range of from about 0.08 to 0.10.

What is claimed is:

1. A method of enhancing the charge acceptance of an electrophotographic imaging member having a photoconductive imaging layer comprising amorphous selenium or selenium alloy,

said method comprising depositing on said imaging layer a charge acceptance effective amount of at least one compound of the formula



wherein R is a saturated aliphatic hydrocarbon radical having from about 8 to about 30 carbon atoms.

2. The method of claim 1 wherein said compound is N-lauryl-morpholine.

3. The method of claim 1, wherein the photoconductive imaging layer comprises a selenium/arsenic alloy.

4. The method of claim 1, wherein the photoconductive imaging layer comprises a selenium/tellurium alloy.

5. The method of claim 1, wherein about 0.2 to about 0.5 micrograms of the above compound is deposited per square centimeter of the surface of the imaging layer.

6. The method of claim 1 wherein a compound of the above formula is first dissolved in a lower alkyl alcohol and the resulting solution applied to the surface of the imaging layer.

7. A method for enhancing the moisture resistance of an electrophotographic imaging member having a photoconductive imaging layer comprising amorphous selenium or selenium alloy,

said method comprising depositing on said imaging layer a moisture resistant effective amount of at least one compound of the formula



wherein R is a saturated aliphatic hydrocarbon radical having from about 8 to about 30 carbon atoms.

8. The method of claim 7 wherein said compound is N-lauryl-morpholine.

9. The method of claim 7, wherein the photoconductive imaging layer comprises a selenium/arsenic alloy.

10. The method of claim 7, wherein the photoconductive imaging layer comprises a selenium/tellurium alloy.

11. The method of claim 7, wherein about 0.2 to about 0.5 micrograms of the above compound is deposited per square centimeter of the surface of the imaging layer.

12. The method of claim 7, wherein the compound of the above formula is first dissolved in a lower alkyl alcohol and the resulting solution applied to the surface of the imaging layer.

13. A method for enhancing the abrasion resistance of an electrophotographic imaging member having a photoconductive imaging layer comprising amorphous selenium or selenium alloy,

said method comprising depositing on said imaging layer an abrasion resistance effective amount of at least one compound of the formula



wherein R is a saturated aliphatic hydrocarbon radical having from about 8 to about 30 carbon atoms.

14. The method of claim 13 wherein said compound is N-lauryl-morpholine.

15. The method of claim 13 wherein the photoconductive imaging layer comprises a selenium/arsenic alloy.

16. The method of claim 13, wherein the photoconductive imaging layer comprises a selenium/tellurium alloy.

17. The method of claim 13, wherein about 0.2 to about 0.5 micrograms of the above compound is deposited per square centimeter of the surface of the imaging layer.

18. The method of claim 13, wherein the compound of the above formula is first dissolved in a lower alkyl alcohol and the resulting solution applied to the surface of the imaging layer.

19. A method for extending the useful life of an electrophotographic imaging member having a photoconductive imaging layer comprising selenium or selenium alloys

said method comprising depositing on said imaging layer a life extending amount of at least one compound of the formula



wherein R is a saturated aliphatic hydrocarbon radical having from about 8 to about 30 carbon atoms.

20. The method of claim 19, wherein said compound is N-lauryl-morpholine.

21. The method of claim 19, wherein the photoconductive imaging layer comprises a selenium/arsenic alloy.

22. The method of claim 19, wherein the photoconductive imaging layer comprises a selenium/tellurium alloy.

23. The method of claim 19, wherein about 0.2 to about 0.5 micrograms of the above compound is deposited per square centimeter of the surface of the imaging layer.

24. The method of claim 19, wherein a compound of the above formula is first dissolved in a lower alkyl alcohol and the resulting solution applied to the surface of the imaging layer.

25. An electrophotographic imaging member comprising a conductive substrate having operatively disposed in relation thereto a photoconductive imaging layer comprising amorphous selenium or selenium alloy, the surface of said imaging layer having deposited thereon a conditioning effective amount of at least one compound of the formula



26. The imaging member of claim 25, wherein said compound is N-lauryl-morpholine.

27. The imaging member of claim 25, wherein the photoconductive imaging layer comprises a selenium/arsenic alloy.

28. The imaging member of claim 25, wherein the photoconductive imaging layer comprises a selenium/tellurium alloy.

29. The imaging member of claim 25, wherein about 0.2 to about 0.5 micrograms of the above compound is deposited per square centimeter of the surface of the imaging layer.

30. An electrophotographic imaging process comprising:

a. providing an electrophotographic imaging member comprising a conductive substrate having operatively disposed in relation thereto a photoconductive imaging layer comprising amorphous selenium or selenium alloy, the surface of said imaging layer having deposited thereon a conditioning effective amount of at least one compound of the formula



31. The process of claim 30, wherein said compound is N-lauryl-morpholine.

32. The process of claim 30, wherein the photoconductive imaging layer comprises a selenium/arsenic alloy.

33. The process of claim 30, wherein the photoconductive imaging layer comprises a selenium/tellurium alloy.

34. The process of claim 30, wherein about 0.2 to

about 0.5 micrograms of the above compound is deposited per square centimeter of the surface of the imaging layer.

\* \* \* \* \*

UNITED STATES PATENT OFFICE  
CERTIFICATE OF CORRECTIONPatent No. 3,860,421 Dated January 14, 1975Inventor(s) Bela Telek and Thomas Skaper

It is certified that error appears in the above-identified patent and that said Letters Patent are hereby corrected as shown below:

Column 2, line 68, change "comprises amorphous selenium alloys" to --comprises amorphous selenium or selenium alloys--.

Column 3, line 36, change "8 to 30" to -- 8 to about 30--.

Column 3, line 42, change "removing" to --removed--.

Column 5, line 8, change "on" to --one--.

Column 5, line 12, change "hydrogen" to --hydrocarbon--.

Column 6, line 40, change "photorecptor" to --photoreceptor--.

Column 6, line 43, change "4,000" to --4000--.

Column 7, line 28 and 29 change "N-caprylym morpholine for N-lauryl-morpholine" to --N-caprylyl-morpholine for N-lauryl-morpholine--.

Claim 1, line 1, change "of" first occurrence to -- for --.

Signed and sealed this 17th day of June 1975.

U.S. PATENT  
OFFICE  
C. MARSHALL DANN  
Commissioner of Patents  
and Trademarks